

# UNITED STATES PATENT OFFICE.

HARLEY T. PECK, OF LEBANON, OHIO, ASSIGNOR TO THE PETERS CARTRIDGE COMPANY, OF CINCINNATI, OHIO, A CORPORATION OF OHIO.

## PRIMER FOR SMALL-ARMS AMMUNITION.

1,407,767.

Specification of Letters Patent. Patented Feb. 28, 1922.

No Drawing.

Application filed December 15, 1919. Serial No. 345,044.

To all whom it may concern:

Be it known that I, HARLEY T. PECK, a citizen of the United States, residing at Lebanon, in the county of Warren and State of Ohio, have invented certain new and useful Improvements in Primers for Small-Arms Ammunition, of which the following is a specification.

This invention has for its object the provision of primers for small arms ammunition which shall be of improved composition and efficiency.

The invention is exemplified in the composition of material described in the following specification, and it is more particularly pointed out in the appended claims.

At present there are two well-known types of small arms primers, namely, center fire and rim fire primers. A center fire primer is composed of a brass, copper or gliding metal cup into which is loaded under pressure the explosive compound which is cemented or held in place by gum, collodion, or some other adhesive, or it may be covered by a paper or tinfoil disc which is held in place by a similar adhesive. The rim fire primers are contained in the head of the cartridge case within the annular rim or cavity provided for this purpose. The priming composition is introduced by means of centrifugal force and projected outwardly from the center into the cavity. It is held in place by gum, collodion, or some suitable adhesive.

Specifically my invention relates to a priming composition of which tri-nitro-resorcinol is an ingredient. Tri-nitro-resorcinol has a chemical formula of  $C_6H(NO_2)_3(OH)_2$ , and is represented graphically by the following formula:



The use of tri-nitro-resorcinol as an ingredient of priming mixtures is specifically designed to provide a primer which will burn in a progressive manner giving a flame

of long duration and intense heat. Tri-nitro-resorcinol as a priming mixture ingredient is superior in that it produces a primer which is more uniform in sensitivity and therefore the tendency to misfire is much more easily controlled than in other primers. Many of the more recently developed smokeless powders which are designed for the purpose of producing a slow rate of combustion and improved ballistics have one fault, namely, that they are difficult of ignition. A primer containing tri-nitro-resorcinol according to the present invention is of such superior quality that it ignites with great ease the latest types of improved progressive powders.

In preparing a primer according to the present invention a priming composition comprising substantially 35% potassium chlorate, 35% fulminate of mercury, and 30% antimony sulphide may be used, to which may be added 5% or more of tri-nitro-resorcinol. Five per cent of tri-nitro-resorcinol is sufficient in most cases to produce the effect desired. If still greater ignition powers are wished a larger amount of tri-nitro-resorcinol may be added. Another priming composition may consist of approximately 5% of tri-nitro-resorcinol added to a rim fire priming composition comprising the following: 40% fulminate of mercury, 40% ground glass, 20% potassium chlorate.

Another composition may include 50% potassium chlorate, 20% antimony sulphide, 30% lead or copper sulphocyanide to which mixture 5% or more tri-nitro-resorcinol is added.

In some cases less than 5% tri-nitro-resorcinol may be used, and the tri-nitro-resorcinol may be added to other priming compositions besides those named above which are given by way of example.

I claim:

1. A priming composition for ammunition containing tri-nitro-resorcinol.
2. A priming composition for ammunition comprising an explosive mixture containing approximately 5% tri-nitro-resorcinol.

3. A priming composition for ammunition comprising a fulminate explosive mixture containing tri-nitro-resorcinol.
4. A priming composition for ammunition comprising a fulminate explosive mixture containing approximately 5% tri-nitro-resorcinol.
5. A priming composition for ammunition comprising an explosive mixture to

which is added tri-nitro-resorcinol to cause 10 the mixture to burn in a progressive manner and to impart uniformity in sensitiveness thereto.

In testimony whereof I have signed my name to this specification on this 9th day of 15 December, A. D. 1919.

HARLEY T. PECK.